

# UNITED STATES PATENT OFFICE.

HERMAN E. BAKKEN, OF NEW KENSINGTON, PENNSYLVANIA, ASSIGNOR TO ALUMINUM COMPANY OF AMERICA, OF PITTSBURGH, PENNSYLVANIA, A CORPORATION OF PENNSYLVANIA.

## PROCESS OF CASTING FREELY-OXIDIZABLE METALS.

1,363,384.

Specification of Letters Patent.

Patented Dec. 28, 1920.

No Drawing.

Application filed January 15, 1920. Serial No. 351,679.

To all whom it may concern:

Be it known that I, HERMAN E. BAKKEN, a resident of New Kensington, in the county of Allegheny and State of Pennsylvania, have invented a new and useful Improvement in Processes of Casting Freely-Oxidizable Metals, of which the following is a specification.

The object of the invention is to provide 10 a process of making castings of freely oxidizable metals whereby the castings will not become oxidized during the casting operation.

While the invention is adapted to the 15 casting of various freely oxidizable metals, such as misch-metal and its constituents, cerium, lanthanum, didymium, etc., it finds particular applicability to the casting of magnesium, and will be so explained in the 20 following description.

Attempts heretofore made to cast magnesium in ordinary molding sand have met with failure due to the fact that the magnesium, when so cast, catches fire and becomes 25 wholly or partially oxidized. This peculiar behavior has been attributed to a reaction between the magnesium and the sand.

My invention is predicated upon my discoveries of the cause of such burning, and 30 of how a clean sound magnesium casting can be made following ordinary foundry practices. I have discovered first that the burning or oxidization of the magnesium is due to the presence of water in the molding 35 sand, the molten metal disassociating the water into its constituent elements and the thus freed oxygen combining with the magnesium; and secondly, that sound clean castings of magnesium can be made by freeing 40 the molding sand of water and rendering it moldable by mixing it with a non-aqueous liquid.

In the practice of the invention, the molding sand may be dried in any desired manner. It is then mixed with sufficient non-aqueous liquid to give it the desired physical properties for molding purposes. While various liquids may be used, such as animal, 45 vegetable and mineral oils, I have found that a heavy petroleum hydro-carbon lubricating oil gives very satisfactory results. After the sand has been thoroughly mixed with, and rendered moldable by the oil, a mold 50 may be made in the usual way, and the mag-

nesium cast into it. The sand may be used 55 repeatedly without the addition of more oil, because little of the oil becomes volatilized or otherwise lost, particularly when a heavy oil is used.

The invention, although particularly useful 60 in green sand molding, is also applicable to dry sand molding in which the molding sand, first freed from water, is mixed with a non-aqueous binder and then molded and baked in the usual manner.

As previously stated, the invention is applicable to the casting of freely oxidizable metals other than magnesium. I desire to have it clearly understood, also, that the invention is not limited to the casting of 70 pure, or even substantially pure, freely-oxidizable metals, but that it is fully applicable to alloys, such as aluminum-magnesium and ferro-cerium alloys, in which the freely-oxidizable metal constituent is present 75 in such proportions as will render the casting liable to destructive oxidization if made in a water-moistened sand mold. Accordingly, the freely-oxidizable metal contemplated in each of the appended claims 80 includes pure metal as well as alloys thereof having oxidizing characteristics similar to the pure metal.

I claim:

1. The process of making a casting of 85 freely oxidizable metal, which consists in forming a mold from sand freed from water and rendered moldable by being mixed with a non-aqueous liquid, and casting said metal in said mold.

2. The process of making a casting of 90 freely oxidizable metal, which consists in forming a green sand mold from sand freed from water and rendered moldable by being mixed with a heavy oil, and casting said metal in said mold.

3. The process of making a casting of 95 freely oxidizable metal, which consists in forming a green sand mold from sand freed from water and rendered moldable by being 100 mixed with a non-aqueous liquid, and casting said metal in said green sand mold.

4. The process of making a magnesium casting, which consists in forming a mold 105 from sand freed from water and rendered moldable by being mixed with a non-aqueous liquid, and casting molten magnesium in said mold.

5. The process of making a casting of a metal containing a considerable proportion of magnesium, which consists in forming a mold from sand freed from water and rendered moldable by being mixed with a non-aqueous liquid, and casting the molten metal in the said mold.

In testimony whereof I have hereunto set my hand.

HERMAN E. BAKKEN.

Witnesses:

FRANCIS C. FRARY,  
H. V. CHURCHILL.